

# United States Patent

[19]

Sakamaki

[11] 3,756,754

[45] Sept. 4, 1973

[54] APEX SEAL FOR ROTARY PISTON ENGINE

3,554,677 1/1971 Zapf et al. .... 418/178

[75] Inventor: Hiroshi Sakamaki, Utsunomiya, Japan

Primary Examiner—Samuel B. Rothberg

[73] Assignee: Nippon Piston Ring Co., Ltd., Tokyo, Japan

Assistant Examiner—Robert I. Smith

[22] Filed: Oct. 21, 1971

Attorney—Sughrue, Rothwell, Mion, Zinn & McPeak et al.

[21] Appl. No.: 191,287

## [57] ABSTRACT

[30] Foreign Application Priority Data

Oct. 24, 1970 Japan..... 45/93840

An apex seal for rotary piston engine has the main body of the apex seal made of a light metal selected from the group of aluminum, aluminum alloy, magnesium, and magnesium alloy with an oxidized layer of more than 10 microns in thickness formed by anodic treatment on at least the sliding surface of the main body, and a heat resistant resin impregnating the oxidized layer.

[52] U.S. Cl..... 418/113, 418/179, 277/235 A  
[51] Int. Cl. .... F01c 19/02  
[58] Field of Search..... 418/113, 120, 122, 418/123, 124, 178, 179; 277/235, 235 A

## [56] References Cited

### UNITED STATES PATENTS

3,608,535 9/1971 Winston..... 418/178

2 Claims, 6 Drawing Figures



PATENTED SEP 4 1973

3,756,754

SHEET 1 OF 2

FIG. 1



FIG. 2 PRIOR ART



**FIG. 3****FIG. 4****FIG. 5****FIG. 6**

## APEX SEAL FOR ROTARY PISTON ENGINE

### BACKGROUND OF THE INVENTION

#### 1. FIELD OF THE INVENTION

This invention relates to an apex seal employed between the rotor and the center housing of a rotary engine.

#### 2. DESCRIPTION OF THE PRIOR ART

Apex seals are mounted on the apex portions of the rotor for ensuring fluid-tightness while the rotor rotates inside the center housing of a multi-circular configuration with the apex seal contacting the inner surface of the center housing. For assuring the fluid-tightness of the apex seal to a satisfactory extent, provisions are made so that the apex seal is heavily depressed onto the inner surface of the center housing not only by a number of springs provided between the rear side of the apex seal and the apex portion of the rotor, but also by the centrifugal force caused by the mass of the apex seal, gas pressure caused by the operational fluid, and the like.

However, because of the excessive depressing force for the apex seal, wear of the apex seal and the inner surface of the center housing is found to be too high, and furthermore, there is a tendency to cause irregular wear on the inner surface of the center housing. Although various reasons cause the irregular wear, the most important is due to the mass of the apex seal.

To be more specific, the frictional force due to the centrifugal force caused by the rotation of the rotor, which appears between the apex seal and the inner surface of the center housing, is increased in proportion to the increase in the mass of the apex seal. Accordingly, the mass of the apex seal must be as small as possible, and, furthermore, the wear resistivity, heat resistivity, and the mechanical strength thereof should be superior because of the fact that the apex seal is slid on the internal surface of the center housing in a heavily depressed manner. When an apex seal made of a carbon alloy, which is widely used, is considered from the above described view point, it is apparent that the apex seal of this kind is not sufficient in mechanical strength as well as in the wear resistivity, and an apex seal satisfying all of these requirements is yet to be found.

#### SUMMARY OF THE INVENTION

Therefore, the primary object of the present invention is to provide an apex seal which can satisfy all of the above described requirements.

This and other objects of the present invention can be achieved by an improved construction of the apex seal which comprises a main apex seal body made of a material selected from a group consisting of aluminum, aluminum alloy, magnesium, and magnesium alloy, at least a sliding surface of the main body of the apex seal being anodized to obtain an oxidized layer of more than 10 microns in thickness, with the anodized layer being either directly impregnated with a heat-resisting synthetic resin or being provided with grooves and then impregnated with the synthetic resin.

The principle, nature, and the utility of the present invention will be better understood from the following detailed description of the invention when read in conjunction with the accompanying drawing.

#### BRIEF DESCRIPTION OF THE DRAWINGS

In the drawing:

FIG. 1 is a vertical sectional view of a rotary piston engine equipped with the apex seal according to the present invention;

FIG. 2 is a perspective view of an apex seal constituting an embodiment of the present invention;

FIG. 3 is a longitudinal sectional view taken along the line III-III in FIG. 2;

FIG. 4 is a longitudinal sectional view similar to FIG. 3 of another embodiment of the present invention;

FIG. 5 is a plan view of still another embodiment of the invention; and

FIG. 6 is a longitudinal sectional view of an apex seal which constitutes still another embodiment of the invention.

#### DETAILED DESCRIPTION OF THE INVENTION

Referring now to FIG. 1, there is indicated a rotary engine comprising a center housing 1 having an internal surface in the form of a multi-circular configuration, side housings 2, 2, a rotor 3 which rotates eccentrically within the center housing 1, a groove 4 provided in each apex portion of the rotor 3 projected adjacent to the internal surface of the center housing 1, an apex seal 5 inserted in the groove 4 so that the seal 5 can be freely moved inside of the groove 4, and a number of springs 6 provided on the rear side of the apex seal 5 for urging the slidable surface 51 of the apex seal 5 onto the internal surface 1' of the center housing 1.

As best seen in FIGS. 2 and 3, the apex seal 5 is made of aluminum, aluminum alloy, magnesium, or magnesium alloy, so that the mass of the apex seal is much reduced despite its high mechanical strength.

However, the apex seal made of aluminum, magnesium, or their alloys has a shortcoming of inferior wear resistivity, and for overcoming the shortcoming, an oxidized layer 7 is formed over the sliding surface 51 of the apex seal 5, which otherwise may be easily worn out, and also on the side surface 52, 52 of the apex seal through an anodic treatment. The thickness of the oxidized layer 7 is selected to be more than 10 microns.

For further imparting wear resistivity and self-lubricating nature, the oxidized layer 7 is impregnated by a heat resistant resin such as fluorocarbon resin or silicone resin.

Alternatively, the sliding surface 51 and the end surfaces 52, 52 may be provided with a number of grooves 9 as shown in FIG. 4, and a wear resistant material 10 such as iron nitride or tungsten may fill the grooves 9. In this case, the shape, orientation, and the number of the grooves 9 may be selected to adapt the type and operation of the rotary engine. For instance, rectilinear grooves 9' may be cut along the length of the apex seal as shown in FIG. 5, and a wear resistant material 10' which is similar to the material 10 may fill the inside of the grooves.

Otherwise, the sliding surface 51 and the end surfaces 52, 52 of the apex seal may be provided with an oxidized layer 7 of more than 10 microns in thickness, the oxidized layer 7 being further impregnated with a heat resistant synthetic resin 8, and a number of grooves 9 may then be provided at least on the sliding surface 51 of the apex seal as shown in FIG. 6. In these grooves 9, a wear resistant material 10 similar to those employed in FIGS. 4 and 5 is placed. In this example, superior wear resistivity can be obtained due to the multiplying effects of the oxidized layer 7, wear resis-

tant synthetic resin 8, and the wear resistant material 10.

As described hereinbefore, the mass of the apex seal of this invention is very small as it is made of aluminum, magnesium, or their alloys, and the mechanical strength thereof is also very high. Furthermore, on the easily wearable sliding surface and the end surfaces of the apex seal, an oxidized layer is formed by way of anodic treatment, which is thereafter impregnated by a heat resistant resin. For this reason, the resultant apex 10 seal is ensured to have superior wear resistivity, self-lubricating nature, and initial affinity.

What is claimed is:

1. An apex seal for a rotary engine comprising: an apex seal main body made of a light metal selected 15 from the group consisting of aluminum, aluminum alloy, magnesium, and magnesium alloy,

an oxidized layer of more than 10 microns in thickness formed by anodic treatment on at least the sliding surface of the main body, and a heat resistant resin impregnating the oxidized layer.

2. An apex seal for a rotary engine comprising: an apex seal main body made of a light metal selected from the group consisting of aluminum, aluminum alloy, magnesium, and magnesium alloy, an oxidized layer of more than 10 microns in thickness formed by anodic treatment on at least the sliding surface of the main body, a heat resistant resin impregnating the oxidized layer, a number of grooves provided at least on the sliding surface of the main body, and a wear resistant material filling said grooves.

\* \* \* \* \*

20

25

30

35

40

45

50

55

60

65